

# UNITED STATES PATENT OFFICE.

GEORG CRUSIUS, OF GROSS-ILSEDE, GERMANY.

## METHOD OF BRIQUETTING IRON ORES AND THE LIKE.

1,116,024.

Specification of Letters Patent.

Patented Nov. 3, 1914.

No Drawing.

Application filed November 29, 1913. Serial No. 803,640.

*To all whom it may concern:*

Be it known that I, GEORG CRUSIUS, a subject of the German Emperor, and resident of Gross-Ilsede, in the German Empire, have 5 invented an Improved and Novel Method of Briquetting Iron Ores and the like, of which the following is a specification.

This invention relates to a method of briquetting iron ores, Thomas slag, residues of 10 such, and particularly also such materials as are not binding *per se*.

The gist of the invention resides in mixing the ores or other material with a tar that has been freed of water and all light and 15 middle oils, the mixed substances being then pressed, as is more fully described hereinafter.

In the briquetting methods employed up to now, either no binding means were made 20 use of, or ordinary tar or soft pitch was used. The employment of these binding means was, however, connected with a variety of drawbacks; for instance, the light and medium oils got distilled off already at 25 very low temperatures so that they had no reducing effect upon the ores and were thus not properly utilized for the smelting process. In fact, the presence of the oils escaping during the process has a noxious effect, 30 because the briquet is made loose and loses consequently in solidity just by the early escape of the oils in question. In contradistinction to this, the iron ores or other materials are treated with tar which is already 35 deprived of water, as well as of the light and the middle oils. This is very advantageous. The oils allow of a highly profitable utilization of their own, whereas the tar product obtained contains solely the heavy oils 40 and remains thinly liquid in spite of that. The thus treated tar is more easily and more intimately mixable with the materials to be briquetted, apart from the further advantage that the heavy oils present within 45 the tar and thus within the mixture get to the outer surface of the briquet during the pressing, soaking the material at the sur-

face, improving thereby the appearance of the briquet, and acting in the mold like a grease thus facilitating removing the 50 finished briquets from the same. The briquets produced in this way are completely weather-proof and resist the heaviest rain, as well as the strongest frost, during being stored, as well as during transport, without the slightest injury whatever. The reductibility of the ores mixed with the tar treated in the manner in question is considerably increased, and coke is saved during the reduction because the tar has carbon 60 as a component and its action and effect are more energetic because of the immediate reduction of the finely divided coke present in the briquet. Also the porosity of the briquets is improved without any damage to 65 their solidity, that increase of the porosity being due to the fact that the briquets when dropping within the blast furnace are freely exposed to the reducing action of the blast furnace gases arising in consequence of the 70 natural coking process of the added tar. (The gases arising act upon the adjacent charge and assist the reducing effect of the blast furnace gases.) Finally, the porous briquets offer the greatest imaginable contact surface whereby the working of the 75 furnace is favorably influenced.

Having now described my invention, what I desire to secure by a patent of the United States is:

The herein described method of briquetting non-binding material which consists in mixing the material with tar which has been deprived of its water, its light oils and its middle oils but which retains its heavy oils, 85 and subjecting the mixture to pressure.

In testimony whereof I have signed my name to this specification in the presence of two subscribing witnesses.

GEORG CRUSIUS.

Witnesses:

KARL GULJAHR.

T. HENDY REED.